

[54] METHOD OF LINING AN EARTHEN TANK

[76] Inventor: Hal K. Jarrell, P.O. Box 4595,  
Odessa, Tex. 79760

[21] Appl. No.: 808,032

[22] Filed: Jun. 20, 1977

[51] Int. Cl. 2 E02B 5/00

[52] U.S. Cl. 52/742; 52/169.7;  
405/270[58] Field of Search 61/1 R, 7, 63, 0.5;  
52/169.7, 169.14, 742, 169.2

## [56] References Cited

## U.S. PATENT DOCUMENTS

|           |         |                 |            |
|-----------|---------|-----------------|------------|
| 2,308,294 | 1/1943  | McCorkle et al. | 61/7       |
| 2,771,745 | 11/1956 | Bramble         | 61/7       |
| 2,887,759 | 5/1959  | Brownell        | 52/169.7 X |
| 3,113,435 | 12/1963 | Yount           | 61/7       |
| 3,160,512 | 12/1964 | Cash et al.     | 61/7 X     |
| 3,474,625 | 10/1969 | Draper et al.   | 61/1 R     |
| 3,849,229 | 11/1974 | Spillane et al. | 61/7 X     |

3,949,113 4/1976 Draper et al. .... 61/1 R

Primary Examiner—Dennis L. Taylor

Attorney, Agent, or Firm—Marcus L. Bates

[57]

## ABSTRACT

A unitary liner for an earthen tank fabricated in situ from a multiplicity of fiberglass panels bonded together to form a unitized membrane which is impervious to brine, crude and drilling mud. The fiberglass panels are prefabricated and rolled into cylinders for delivery to the tank site where field fabrication of the membrane is completed by attaching overlapping edges of the panels to one another to form a seam. The edges are subsequently bonded together by fiberglass cloth and polyester resin. The fiberglass panels are made up of a plurality of sheets of paper and fiberglass cloth bonded together by fiberglass resin. The cylinder is of a configuration which enables it to be easily handled by workmen.

10 Claims, 12 Drawing Figures



FIG. 1



FIG. 2



FIG. 3



FIG. 4



FIG. 5



FIG. 6A





## METHOD OF LINING AN EARTHEN TANK

## BACKGROUND OF THE INVENTION

During the drilling of boreholes, such as occasioned in seeking oil and gas production, the drilling rigs must have made available a nearby large storage pond, called a mud pit, so that drilling mud can be mixed with various different chemical additives in order to carry out a proper drilling operation. Brine is often used in tremendous quantities in drilling operations and the handling of thousands of gallons of salt water is costly and must be carefully contained in order to avoid waste and contamination of the immediate area. It is especially important that the brine be contained within a reliable storage pond or tank in order to prevent damage to the underlying aquifer as may occur by the salts and chemicals escaping through the tank bottom and soaking into the fresh water zone. Moreover, vegetation, livestock, and wild animal life must be protected from runoff and spillage of the various chemicals employed in drilling a borehole.

Heretofore, the importance of lining earthen tanks has been ignored, or else the tanks have been inadequately lined by cementing together the edges of several polyethylene sheets. This is difficult to properly carry out in the field because the wind blows the light weight polyethylene about, making it difficult to effect a proper bond at the seams; and, furthermore, dirt and debris is blown onto the glue, causing the seam to subsequently part. The polyethylene liner is easily damaged by rocks and other sharp objects. Moreover, air entrapped under the plastic liner tends to float the entire liner to the surface, and therefore, it is not unusual for the workmen to attempt to overcome this drawback by throwing weights, rocks and other debris into the tank. Of course, this action contributes to the danger of injuring the liner as well as contaminating the contents of the tank.

Therefore, it is desirable to have a tank liner in the form of a unitary membrane which is impervious to drilling mud, chemical additives, and salt water. It would be desirable that the membrane be efficiently fabricated insitu to form a monocoque liner which overcomes the above drawbacks and which is not easily damaged.

## SUMMARY OF THE INVENTION

This invention relates to tank liners and specifically to a method of lining an earthen tank with a unitary plastic impregnated fiberglass membrane by bonding fiberglass and paper together with a polyester resin to form a panel. The panel is rolled up into a convenient cylindrical roll and transported to the tank site.

The tank is formed by an excavation made into the ground and the panels are unrolled and placed within the tank adjacent to one another with the marginal edges thereof overlapping one another. The overlapped edges are bonded to one another by utilizing polyester resin and fiberglass cloth to thereby effect a unitary membrane which completely covers the entire bottom of the tank.

The marginal peripheral edges of the membrane preferably extends horizontally away from the tank and an overburden of earth is placed thereon to protect the marginal edges of the liner from livestock and equipment.

A primary object of the present invention is the provision of a unitary tank liner fabricated insitu and made of individual fiberglass panels having the edges thereof bonded to one another.

5 Another object of the invention is to provide a resin impregnated unitary fiberglass membrane for lining an earthen tank.

10 A further object of this invention is to disclose and provide a tank liner fabricated insitu by special fiberglass panels joined together to provide a unitary membrane which is impervious to salt water and drilling mud.

15 A still further object of this invention is to provide a polyester impregnated fiberglass tank liner made by field joining a multiplicity of panels together to provide a unitary membrane for containing liquids within an earthen tank.

20 The above objects are attained in accordance with the present invention by the provision of a combination of elements which are fabricated in a manner substantially as described in the above abstract and summary.

25 These and various other objects and advantages of the invention will become readily apparent to these skilled in the art upon reading the following detailed description and claims and by referring to the accompanying drawings.

## BRIEF DESCRIPTION OF THE DRAWINGS

30 FIG. 1 is a cross-sectional view taken along line 1—1; of FIG. 2 and discloses a tank having a liner made in accordance with the present invention;

35 FIG. 2 is a plan view of a tank having a liner made in accordance with the present invention;

FIG. 3 is an enlarged, broken, top plan view which discloses the tank of FIGS. 1 and 2 under construction;

FIG. 4 is a cross-sectional view taken along line 4—4 of FIG. 3;

FIG. 5 is a top plan view of part of the tank liner apparatus disclosed in FIGS. 1-3.

40 FIG. 6A is a cross-sectional view taken along line 6—6 of FIG. 5 and FIG. 6B is a modification thereof;

FIG. 7 is an end view disclosing the material of FIG. 5 in a rolled up configuration;

45 FIG. 8A is a cross-sectional side view of the tank lines of the present invention and FIG. 8B is a modification thereof.

FIG. 9 is a cross-sectional view taken along line 9—9 of FIG. 8; and,

50 FIG. 10 is a cross-sectional view of another embodiment of this invention.

## DETAILED DESCRIPTION OF THE PREFERRED EMBODIMENTS

FIG. 1 discloses a tank 10 formed into the earth and 55 adapted to hold salt water, crude oil, alkali solution, drilling mud, or various other chemical products. The area 12 surrounding the tank generally slopes downwardly therefrom with an embankment 14 usually being formed about the outer periphery of a tank liner 16 made in accordance with the present invention. Numeral 18 indicates the liquid level of the tank. The outer marginal peripheral edge portion 20 of the tank liner lies horizontally and preferably is covered with earth in the indicated manner of FIGS. 1 and 2.

The tank liner 16 is a unitary membrane and comprises a multiplicity of parallel panels 22 made in accordance with the present invention. The corners 24 of the tank may be at an abrupt angle as illustrated, or alterna-

tively may be smoothly contoured into a long sweeping curve, as may be desired.

FIG. 3 discloses the method of fabricating the tank liner 16. As illustrated, the elongated, parallel, adjacent panel members 22 are arranged with their adjacent edges 25 and 26 slightly overlapping one another, as for example 2 or 3 inches of overlap for a panel of material 10 or 20 feet in width.

Numerical 27 indicates the step of placing a panel of material 22' adjacent to panels of material 22 already formed into the tank liner. The material of sheet 22' is laid down by unrolling the rolled up cylinder of material 122.

Numerical 28 indicates a reinforced lap-joint made insitu in accordance with the present invention. The lap-joint is formed by sand blasting the overlap area in the indicated manner of numeral 30 by employment of sandblasting equipment 32 having an outlet nozzle 34 of conventional design. Numerical 36 indicates plastic resin which has been applied to the sandblasting area.

As seen in FIGS. 3 and 4, the roll of material 122 is unrolled and panel 22' properly overlapped respective to the last laid panel, whereupon the adjacent panels are attached to one another by staples 38. Numerical 40 indicates a six inch width of reinforcement fiberglass matt bonded to the margins of two adjacent panels to reinforce the seam 28. Numerical 42 shows the fiberglass resin which is applied to complete the seam 28.

In FIGS. 5 and 6, numerals 44 and 46 indicate two sheets of material which are joined together to form a panel. Numerical 48 indicates a joint where reinforced material is placed at the longitudinal interseam 50 for effectively bonding the individual sheets of material together during the manufacture thereof.

Each sheet of the panel of material comprises a lower layer 52 of craft paper, a layer of fiberglass matt 54, which preferably is 1½ ounces per square foot, and is available from Fiberglass Inc., Garland, Texas, with polyester resin 56 and 58 forming the outer surface. The polyester resin is a special blend comprised of iso and artho polyesters which impart flexibility into the panels and is available from Cook Paint and Varnish Company, Kansas City, Kas.

The outer surface adjacent the interface 58 is not sand blasted for the reason that the fiberglass reinforcing strip 60 is affixed to the outer surface of the panel with fiberglass resin 62 before the polyester resin 56 has completely cured.

The panels preferably are comprised of two 100 feet lengths of 5 feet wide fiberglass sheets which results in a, 100' × 10' panel. The panel can be rolled into a cylinder 122 is illustrated in FIGS. 3 and 7.

FIGS. 8 and 9 set forth in the constructional details of the completed tank liner. As seen in FIGS. 8A and 9, the factory splice 48 joins a plurality of sheets together to provide a multiplicity of panels which are joined together by a field splice 28 so that the tank liner comprises a membrane fabricated insitu in accordance with the method of the present invention.

FIGS. 6B and 8B illustrates another embodiment of the invention wherein the individual panels are fabricated from sheets having the marginal adjacent edges thereof overlapped and bonded together. The papers 52, 53 are overlapped and bonded to the overlapped 65 fiberglass sheets 54, 55. Polyester 44 and 46 forms the outer surface and completes the panel. Numerical 148 broadly indicates the factory lap seam.

As particularly seen in FIG. 8B, the panels 22' are joined together at 28 in the same manner described above in conjunction with FIG. 8A. The field seams 28 join the panels 22' together to form the tank liner or continuous membrane.

FIG. 10 illustrates a large storage tank 68 having a bottom 70 therein which has been aged at 72 whereupon it will no longer hold liquid and the entire bottom heretofore usually must be replaced. A roof 74 is supported by the tank sidewalls 76 in the usual manner.

The bottom of the tank is repaired in the manner indicated by numeral 78 by providing a monolithic new plastic floor therewith in accordance with the present invention. The new floor is comprised of spraying foam plastic material 80 to a depth of 2-4 inches into the bottom of the tank with the foam bottom being carefully applied so as to achieve a smooth level floor. Inlet and outlet holes are marked so that they can be opened later on. A layer of rubber, like material 66 of about ½ inch in thickness is next applied over the entire surface of the floor. The rubber-like material is made of Urethane plastics which air dries to provide a resilient, impervious, continuous tank bottom. The rubber-like material can also be catalyst cured as is known to those skilled in the art.

In carrying out the method of the first embodiment of the present invention, a plurality of sheets of craft paper are laid in side by side abutting relationship and extended in width and length in an amount slightly greater than the panel being fabricated. The paper preferably comprises two parallel sheets six feet in width thereby providing ample overage which can be trimmed from the final panel.

Two adjacent abutting sheets of fiberglass matt five feet in width and one hundred feet in length are laid out in superimposed relationship on the paper with the adjacent edge portions of the fiberglass matt abutting one another. Polyester resin is next sprayed onto the matt and the narrow strip of material 60 is next applied before the polyester resin has set up. Additional polyester resin is applied to the strip 60 by using special paint rollers having a nap cover thereon made especially for the fiber glass industry.

As soon as the fiberglass resin has cured to hardness, which normally is about one hour, the excess paper is trimmed from the edges and the panels are stacked for final cure which requires 1-3 days, depending upon the temperature, humidity and ventilation. The finally cured panels are each rolled into a cylinder 122 and stored until needed to fabricate the tank.

In the second embodiment of the invention disclosed in FIGS. 6B and 8B, the craft paper is laid out on the floor in the before described manner but with the adjacent longitudinal edge portions thereof being overlapped as seen in FIG. 6B at numeral 148. When the sheets of matt are superimposed upon the craft paper, care is taken to overlap the adjacent edges thereof approximately two inches, thereby eliminating the need for the strip of reinforcing matt 60 illustrated in FIG. 6A. The panels are cured and rolled in cylinders as in the before described manner.

The tank site is prepared by excavating a suitable area and using the excavated material to build up the sides thereof. Padding material, such as chip base or sand, is added as needed to made absolutely certain that a suitable bed is presented for receiving the unitary membrane. The rolls of material are next unrolled in the illustrated manner of FIG. 3 and the overlapping edges

25, 26 thereof stapled using a commercial air stable gun, as seen at 38 in FIGS. 3 and 4. In order to properly bond each of the panels to one another, it is essential that the area 30 be sandblasted so as to remove objectional films of material therefrom and furthur to roughen up an area which is to receive the fiberglass resin, thereby enhancing the bond. The resin and strip 40 is applied at the interface by utilizing the aforementioned roller.

After the membrane has been fabricated insitu a portion of the excavating material is back filled at 14 10 thereby covering the marginal peripheral edge portion of the membrane to prevent future damage thereto.

The present invention provides a unitized membrane which lines an earthen tank in an improved and unusual manner and thereby prevents leakage of objectionable 15 chemicals into the surrounding area.

I claim:

1. Method of lining an earthen tank with a unitary membrane comprising the steps of:

laying down sheets of paper to form a backing for one 20 of a multiplicity of panels;

laying down a plurality of sheets of fiber glass material on said backing with adjacent longitudinal edges of the sheets contacting each other;

impregnating the fiber glass material with polyester 25 resin thereby bonding the material to the paper;

reinforcing the adjacent marginal edges of the sheets of fiber glass with an overlay of fiber glass material and impregnating the overlay with polyester resin; curing the panel and thereafter rolling the panel into 30 a cylinder;

transporting a multiplicity of the cylinders to an earthen tank;

unrolling the panels while overlapping the marginal edges thereof and temporarily fastening the overlapping edges together;

bonding the panels together by applying a strip of fiber glass material impregnated with polyester resin at said overlap;

continuing to add additional panels to cover to bottom and sidewalls of the earthen tank until the tank is completely lines with the panels each being bonded to one another to thereby form a unitary build up fiber glass membrane which is impervious to drilling mud and brine.

2. The method of claim 1 and further including the step of sandblasting a marginal width of the adjacent panels at said overlap prior to bonding the adjacent panels to one another.

3. The method of claim 2 wherein the adjacent panels are temporarily fastened by using staples to fasten the panels to one another prior to the bonding step.

4. The method of claim 3 wherein the marginal peripheral edges of the membrane are made to extend horizontally away from the tank and further including the step of placing an overburden of the earthen mate-

rial thereon to thereby protect the marginal peripheral edge portion of the tank liner.

5. The method of claim 1 wherein the adjacent sheets of fiber glass are limited to two sheets which are five feet wide and one hundred feet in length, and which are joined together to form a ten foot panel one hundred feet in length.

6. The method of claim 1 and further including the step of stapling the overlapping edges of said panels to one another at spaced intervals along the overlapped edges thereof; and,

sandblasting the marginal area of each sheet adjacent to said overlap;

thereby improving said bond.

7. Method of lining an earthen tank with a unitary membrane comprising the steps of:

1. laying down sheets of fibrous material, such as paper, to form a backing for one of a multiplicity of panels;

2. building up a layer of fiberglass material which is supported in superimposed relationship on said backing; and,

3. impregnating the layer of fiberglass material with polyester resin, thereby bonding the fiberglass material, polyester resin, and fibrous material together to form said panel;

4. curing the panel and thereafter rolling the panel into a cylinder;

5. transporting a multiplicity of said cylinders to an earthen tank;

6. unrolling the panels and bonding the adjacent edges of adjacent panels together by applying fiberglass material impregnated with polyester resin at said adjacent edges;

7. repeating step (6) in order to add additional panels to cover the bottom and sidewalls of the earthen tank until the tank is completely lined, with the panels each being bonded to one another to thereby form a unitary build-up fiberglass membrane which is impervious to drilling mud and brine.

8. The method of claim 7 and further including the step of sandblasting a marginal width of the adjacent panels prior to bonding the adjacent panels to one another.

9. The method of claim 8 wherein the adjacent panels are temporarily fastened to one another by using staples to fasten the panels to one another prior to the bonding step.

10. The method of claim 9 wherein the marginal peripheral edges of the membrane are made to extend horizontally away from the tank and further including the step of placing an overburden of earthen material thereon to thereby protect the marginal peripheral edge portion of the tank liner.

\* \* \* \* \*

UNITED STATES PATENT OFFICE  
CERTIFICATE OF CORRECTION

Patent No. 4,125,983 Dated November 21, 1978

Inventor(s) HAL K. JARRELL

It is certified that error appears in the above-identified patent and that said Letters Patent are hereby corrected as shown below:

Line 54, delete "in" after forth.

Line 60, substitute --into-- for "in";  
Line 65, substitute --make-- for "made".

Column 5, line 40, substitute --the-- for "to", second occurrence;

Line 42, substitute --lined-- for "lines";  
Line 44, substitute --built-- for "build".

Column 6, line 40, substitute --built-up-- for "build-up".

Signed and Sealed this

*Twenty-sixth Day of June 1979*

[SEAL]

Attest:

RUTH C. MASON  
*Attesting Officer*

DONALD W. BANNER  
*Commissioner of Patents and Trademarks*